

## 1

3,109,917

## HARD FACING

Alfred Schmidt and Erich Nonninger, Kapfenberg, Styria, Austria, assignors to Gebr. Böhler & Co. Aktiengesellschaft, Vienna, Austria  
 No Drawing. Filed Apr. 11, 1960, Ser. No. 21,083  
 Claims priority, application Austria Apr. 18, 1959  
 2 Claims. (Cl. 219—76)

It has been wellknown, that cemented carbides can be welded in inert-gas-atmosphere either with or without admixes of auxiliary metals; this process has proved especially successful in built-up-welding for making tools with cutting-edges. In this process also rods, containing cemented-carbides can be used as admixes.

As far as preparing of wear-resistant surfaces is concerned, this method only could be applied for relatively small surfaces, i.e. surfaces of but a few square-cm., armor-platings on greater surfaces being sensible towards crack-formation and being likely to chip off if exposed to impact-stresses.

This invention deals with an improvement of that well-known process, enabling armor-plating of greater surfaces, especially of round pieces entirely homogeneously, without any crack-formation involved.

Experiments have shown, that the auxiliary metal used for preparing admixes of sintered-carbides is very important. The auxiliary metal used for those admixes is supposed to contain 5—100% Ni, 0—95% Fe and/or 0—30% Cr.

Thus this invention relates to a process of preparing hard and wear-resistant surfaces by built-up-arc-welding in inert gas-atmospheres, whereas admixes of sintered carbides are used, which primarily consists of tungsten-carbides which may be combined with other cemented carbides and of 5—30% auxiliary metal; this process is characterized by the fact, that the auxiliary metal used for armor-plating great surfaces, which are sensible towards crack-formation, especially for armor-plating round pieces, consists of 5—100% Ni, 0—95% Fe and/or 0—30% Cr, besides unavoidable impurities.

Besides tungsten-carbide, which is supposed to be the main component, its percentage being supposed to exceed 50%, carbides of molybdenum, chromium, tantalum, niobium, titanium, zirconium and similar can also be used.

The auxiliary metal either can be pure nickel-powder or nickel-powder mixed with powdered iron or chromium; this auxiliary metal is added to the powdered mixture, which is to be sintered and to be pressed for preparing the admix.

Powdered austenitic Cr-Ni-steel, however, also can be applied as auxiliary metal.

Admixes preferably are made in the usual manner: the powdered mixture, consisting of cemented carbides and binding-metal is mixed with an organic binding-agreant, such as synthetic resin; this mixture is extruded to rods, which subsequently are sintered at temperatures ranging between 900 and 1300° C.

Welding-rods consisting of 85% WC and 15% Ni for

## 2

instance have been used for armor-plating rings for wire-rod-guides according to the process suggested by this invention. No wear could be observed on those rings after 478 hours' running-time. However rings, armor-plated with hardened punching-tool-steel, containing 13% chromium and 2% carbon already have become completely worn out and therefore unable for use, after 334 hours if exposed to the same amount of stress.

If cobalt and/or iron are used as binding-metals the resistance towards wear will be presumably reduced by at least 20% under comparable conditions.

If admixes as suggested by this invention are used for welding in inert atmospheres, hardnesses ranging between 64 and 67 Rockwell-units are achieved. The favourable

15 effect of binding-metals added to those admixes evidently is due to formation of a viscous transition-zone between the admix and the basic material. This enables continuous building up of thicker layers without any crack-formation involved during argon arc-welding. Those layers 20 can have thicknesses ranging between 4 and 6 mm. It is also possible to apply several layers by built-up-welding without any crack-formation involved.

Those admixes as specified by the invention besides have proved especially advantageous owing to the fact, that in 25

argon-arc-welding hardnesses ranging between 64 and 67 RC immediately can be achieved, whereas hardnesses of about 52 RC only are achieved, with the same welding-process, if sintered carbides, such as WC is used with Co and/or Fe as binding-metal.

30 What we claim is:

1. A process of hard facing by shielded arc welding employing a hard facing sintered rod produced by molding and sintering at a temperature of 900—1300° C. an admixture of powdered materials comprising a major portion of hard metal carbides and 5% to 30% of a cobalt free alloy consisting essentially of a metal selected from the group consisting of nickel, iron and chromium and mixtures thereof, at least 5% nickel being present in the alloy and less than 30% chromium being present in the alloy and an organic synthetic resin as a binding agent.

2. The process of claim 1 wherein the hard metal carbide is tungsten carbide.

## References Cited in the file of this patent

## UNITED STATES PATENTS

|           |                |       |               |
|-----------|----------------|-------|---------------|
| 1,721,416 | Schröter       | ----- | July 16, 1929 |
| 1,977,361 | Taylor et al.  | ----- | Oct. 16, 1934 |
| 2,002,198 | Wissler        | ----- | May 21, 1935  |
| 2,067,166 | Balke          | ----- | June 12, 1937 |
| 2,137,471 | Zublin         | ----- | Nov. 22, 1938 |
| 2,219,462 | Wissler        | ----- | Oct. 29, 1940 |
| 2,507,195 | Colbeck et al. | ----- | May 9, 1950   |
| 2,847,555 | Yenni          | ----- | Aug. 12, 1958 |
| 2,982,845 | Yenni et al.   | ----- | May 2, 1961   |
| 2,998,922 | Gibson         | ----- | Sept. 5, 1961 |

## FOREIGN PATENTS

|         |               |       |               |
|---------|---------------|-------|---------------|
| 395,721 | Great Britain | ----- | July 7, 1933  |
| 592,214 | Canada        | ----- | Feb. 9, 1960  |
| 732,440 | Great Britain | ----- | June 22, 1955 |